

W. McCONWAY.

METHOD AND APPARATUS FOR THE PRODUCTION OF CAST STEEL BLANKS.

APPLICATION FILED JUNE 5, 1915.

1,177,957.

Patented Apr. 4, 1916.

2 SHEETS—SHEET 1.



William McConway  
By Ritter & Ritter  
His Attorneys

W. McCONWAY.

METHOD AND APPARATUS FOR THE PRODUCTION OF CAST STEEL BLANKS.

APPLICATION FILED JUNE 5, 1915.

1,177,957.

Patented Apr. 4, 1916.

2 SHEETS—SHEET 2.



Inventor

William McConway  
By *Peter & Peter*

Attorneys

# UNITED STATES PATENT OFFICE.

WILLIAM McCONWAY, OF PITTSBURGH, PENNSYLVANIA.

## METHOD AND APPARATUS FOR THE PRODUCTION OF CAST-STEEL BLANKS.

1,177,957.

Specification of Letters Patent.

Patented Apr. 4, 1916.

Application filed June 5, 1915. Serial No. 32,379.

*To all whom it may concern:*

Be it known that I, WILLIAM McCONWAY, a citizen of the United States, residing at Pittsburgh, in the county of Allegheny and State of Pennsylvania, have invented certain new and useful improvements in Methods and Apparatus for the Production of Cast-Steel Blanks; and I do hereby declare the following to be a full, clear, and exact description of the invention, such as will enable others skilled in the art to which it appertains to make and use the same.

My invention relates to the production of steel blanks from the molten metal, and has for its object the prevention of cracks in and on the periphery of the casting.

Heretofore, when practising the ordinary methods of vertical casting in stationary molds, attempts have been made to prevent the formation of cracks in and on the exterior surface of the casting by applying pressure to the casting in the mold after the casting has sufficiently cooled to form a solid shell around the inclosed molten metal, and in the practice of such method the use of expandible molds has also been suggested. In the practice of what is termed centrifugal casting it has been proposed, in the production of hollow cylindrical castings, to

employ a mandrel or roller, within the hollow cylindrical casting and extending longitudinally thereof, with intent to solidify and compact the metal and smooth the interior of the casting; but such a method results in a violent disturbance of the molecules of the steel at a critical period in cooling and so degrades the quality of the metal.

My present invention relates more particularly to what is termed centrifugal casting wherein the molten metal is delivered, when in a high state of fluidity, directly to a rotating mold, the axis of rotation being horizontal, whereby the molten metal is instantly distributed to the peripheral lines and there remains *in situ* until solidified as hereinafter shown. As the centrifugal method of casting is at present practised the tendency of the metal in the matrix to contract is opposed to the centrifugal force incident to the rotation of the mold, with the result that there is a tendency of the casting to withdraw from the face of the mold or matrix in a direction opposed to the direction of operation of the centrifugal force, and this is productive of peripheral cracks in the casting. To meet these con-

ditions in the centrifugal casting of steel, I have devised a method which involves the application of continuous pressure to the revolving molten metal in a direction normal to the centrifugal force during the casting operation, and the maintenance of said pressure continuously until the casting has sufficiently solidified to retain its form when in a quiescent state, after which the centrifugal force and pressure on the casting are discontinued and the normal cooling and contraction thereof is allowed to proceed; and such a method involves the main feature of my invention. For the purpose of carrying out this method I have devised a centrifugal mold which is adapted for the direct reception of the molten steel and which has a hydrostatically driven plunger whereby continuous pressure of adequate force, to be governed by the mass of the casting, may be applied to the casting longitudinally with the axis thereof, or normal to the direction of operation of the centrifugal force during the granulating period of the casting; and a centrifugal casting apparatus thus constructed to be capable of being operated to produce such an effect, involves a secondary feature of my invention.

In the drawings chosen for the purpose of illustrating an apparatus adapted to be utilized in carrying out my improved method of centrifugal casting, Figure 1 is a side elevation of centrifugal casting apparatus embodying my invention. Fig. 2 is an elevation of the charging end of said apparatus. Fig. 3 is a longitudinal vertical section of the apparatus shown in Fig. 1; and Fig. 4 is a longitudinal vertical section of a modified form of the apparatus.

Like symbols refer to like parts wherever they occur.

I will now proceed to describe my invention more fully so that others skilled in the art to which it appertains may apply the same; and as an understanding of the character of the devices necessary to the carrying out of the method will, it is believed, tend to a better comprehension of the method itself, and serve to more clearly differentiate my method from the prior art, I will first describe the apparatus employed by me.

In the drawings, 1 indicates a cylindrical mold adapted for the production of hollow cylindrical castings or ingots C. This mold

is horizontally disposed and is secured by bolts 1<sup>b</sup>, or otherwise, to a revolving disk or head 2 having a centrally disposed, hollow trunnion or shaft 3, the opposite end of 5 which shaft or trunnion 3 is also provided with a disk or head 4 constituting one head of a cylinder 5. The hollow shaft or trunnion 3 is journaled in bearings on a pedestal 6. The opposite head 7 of the cylinder 5 is 10 also provided with a hollow trunnion 8 that is in axial alignment with the hollow shaft or trunnion 3, and said trunnion 8 is journaled in bearings on a pedestal 9.

The outer end of hollow shaft or trunnion 15 8 is closed by a head or disk 10 secured thereto by bolts 11, or in other suitable manner, and said head has a central opening and gland 12 through which passes a pipe 13 that is connected to a pump or other 20 source of hydrostatic pressure. The inlet pipe 13 for hydrostatic pressure is axially disposed with relation to the hollow shaft or trunnion 8 and is held in stationary position in its axial relation to the shaft by 25 means of an arm or bracket 9<sup>b</sup> on the pedestal 9.

Within the cylinder 5 is a piston 14 whose stem 15 extends through the hollow shaft or trunnion 3 and into the mold 1, and 30 which is provided within the mold with a head or piston 16, of a diameter substantially equal to the interior diameter of mold 1. These devices form a convenient means for applying continuous pressure to the casting in the mold during the rotation of said mold. The periphery of the cylinder 5 constitutes and is in effect a pulley 5<sup>a</sup> mounted on the shaft 3, whereby the mold 1 may be rotated from a suitable source of power 35 through the medium of a belt passing around such pulley.

The outer end of the rotatable mold 1 is formed as a disk or head 17 which is secured on the mold and to the revolving head 2 by 45 bolts 18, and said disk or head 17 is provided with a centrally disposed opening or throat 19 through which extends the lower end of a funnel or spout 20 by means of which the molten metal is introduced into 50 the rotatable mold 1 at the time of casting.

In the modified form of the apparatus shown in Fig. 4 of the drawings, the cylindrical mold 1<sup>a</sup>, the revolving head 2<sup>a</sup>, the hollow shaft 3<sup>a</sup>, the pedestals 6<sup>a</sup> and 9<sup>a</sup> in 55 which the hollow shaft 3<sup>a</sup> is journaled, the head or piston 16<sup>a</sup> within the mold and the stem or piston rod 15<sup>a</sup>, which extends through the hollow shaft 3<sup>a</sup>, each and all have their counterparts in similar relations 60 in the preferred form of the apparatus shown in Figs. 1 and 3 of the drawing. But in lieu of applying the continuous pressure to the casting by hydrostatic pressure, which requires a cylinder and piston, there has 65 been substituted for these last named ele-

ments a pointed pressure screw 21 which is supported in axial alignment with the stem 15<sup>a</sup> of the piston head 16<sup>a</sup> by means of a bracket or arm 9<sup>c</sup> on the pedestal 9<sup>a</sup>. The hollow shaft 3<sup>a</sup> is provided with a pulley 3<sup>b</sup> 70 for rotating the shaft and mold.

In carrying out my method of centrifugal casting with an apparatus of the character hereinbefore described I proceed as follows: The rotatable mold having been set in motion to enable it to exert such centrifugal force on the molten contents thereof as will maintain the molten metal in contact with the walls of the mold which a peripheral speed of approximately sixty-five feet per second or upward will suffice to accomplish, the molten steel in a high state of fluidity is introduced into the mold and as soon as the congelation of the metal sets in a progressive pressure is applied longitudinally 80 of the casting or, in other words, normal to the direction or operation of the centrifugal force induced by the rotation of the mold. The application of this progressive force, which may be effected by a continuing application of power to the follower or piston 16 (or 16<sup>a</sup>) that traverses the mold, is continued until the casting has reached the point of solidification where it will maintain its form in a quiescent state, when the 95 rotation of the mold is arrested and the pressure on the piston (16 or 16<sup>a</sup>) is released, thus relieving the casting of the pressure of both the centrifugal force and the force normal thereto. The casting is 100 then permitted to cool in the usual manner, being then subject only to the force of contraction incident to cooling. The progressive pressure thus applied to the casting in a direction normal to the centrifugal force 105 during the formative or granulating period when the contraction in the casting due to cooling is opposed by the centrifugal force causes the casting to be compressed longitudinally and to expand diametrically so as 110 to maintain the contact of the periphery of the casting with the walls of the matrix and prevent the formation of peripheral cracks in the casting. It is to be noted that when the pressure is in excess of that required to maintain steady peripheral contact with the matrix the excess of pressure becomes circumferential and prohibits 115 molecular separation.

Having thus described my invention, 120 what I claim and desire to secure by Letters Patent is:

1. The method of producing steel blanks from molten steel which involves the simultaneous subjection of the molten steel to the 125 operation of centrifugal force and to a force applied in a direction normal to said centrifugal force.

2. The method of producing steel blanks from molten steel which involves the simul- 130

taneous subjection of the molten steel to the operation of centrifugal force and to uniform pressure normal thereto.

3. The method of producing steel blanks 5 from molten steel involving the simultaneous subjection of the molten steel to the operation of centrifugal force and to a force acting normal thereto during the formative period of the blank and discontinuing the 10 application of said forces when the molten metal has solidified to a point where the blank will retain its shape when quiescent.

4. In apparatus for casting blanks from molten steel, the combination with a rotatable mold, of means progressively movable 15 in the axial line of the mold for exerting positive pressure on the molten metal in the mold.

5. A method of producing cast steel blanks 20 which involves the subjection of the molten mass during its granulation to the action of

forces the directions of which are normal to each other.

6. The method of forming a cast steel annulus which involves subjecting a mass of 25 molten steel to centrifugal force and applying a compressive force to the mass of metal in direction of length of the annulus during granulation of the steel.

7. In apparatus for casting blanks from 30 molten steel, the combination with a rotatable mold, of means for rotating the mold to exert centrifugal force on the molten metal during the casting thereof, and means within the mold and movable axially of the 35 mold to exert on the molten metal a force normal to the centrifugal force created by the rotation of the mold during the casting operation.

In testimony whereof I affix my signature. 40

WILLIAM McCONWAY.